

April 23, 1946.

H. R. DALTON ET AL

2,398,779

METHOD OF MAKING DUPLICATING BLANKS BY TELEFACSIMILE AND THE LIKE

Original Filed March 24, 1942



HAROLD R. DALTON  
AUSTIN G. COOLEY  
INVENTORS

BY *John J. Logan*  
ATTORNEY

Patented Apr. 23, 1946

2,398,779

# UNITED STATES PATENT OFFICE

2,398,779

## METHOD OF MAKING DUPLICATING BLANKS BY TELEFACSIMILE AND THE LIKE

Harold R. Dalton, Teaneck, N. J., and Austin G. Cooley, New York, N. Y., assignors, by means assignments, to Timefax Corp., Philadelphia, Pa., a corporation of Pennsylvania

Original application March 24, 1942, Serial No. 435,944. Divided and this application March 24, 1943, Serial No. 480,286

7 Claims. (Cl. 178—6.6)

This invention relates to recording mediums and more particularly to recording blanks such for example as those used for recording electrical signals whether facsimile signals, telegraph signals, sound signals or the like which are to be translated into visible recordings.

Heretofore, numerous kinds of facsimile recording blanks have been proposed which are roughly divisible into two categories, viz., the light sensitive or photographic blank, and the electro-chemical or electromechanical blank. While blanks of both categories have achieved success under conditions of use peculiar to each respectively, they both suffer from the limitation of requiring elaborate and comparatively slow procedure and equipment if a large number of copies are to be made of the subject matter recorded on the blank. Under certain conditions of use, it is quite desirable, upon the receipt of intelligence on a facsimile blank, that this intelligence be capable of duplication as soon as possible after receipt and with a maximum of legibility or readability. In the case of transmission of messages or intelligence by telefacsimile, it is in some cases not possible, or advisable, to repeat the facsimile transmission and yet it may be necessary to use the single facsimile record as a master to control the production of a very large number of duplicate imprints. It should also be remembered that there are rather rigid requirements for the telefacsimile recording blank itself in order that the message or intelligence can be satisfactorily recorded from the electric signals. Bearing in mind these various requirements, we have devised a facsimile record blank which does not sacrifice any of its sensitivity or accuracy as a direct recording blank for received facsimile signals, and which can also be used substantially immediately as a matrix or master record to transfer or imprint a very large number of duplicates.

After consideration of the following disclosure, it will be apparent that while the invention finds its greatest immediate utility in the field of telefacsimile transmission, the fundamental inventive concept is capable of adaptation directly to other fields such as telegraph systems, sound recording systems, motion picture systems (e. g., animated cartoons), and in fact any field wherein the master copy is required to reproduce a large number of duplicates by a non-photographic process.

Accordingly, it is a principal object of the invention to provide a novel method of recording electric signals by employing a recording blank having a plurality of layers of material so that when the blank is subjected to an electric discharge thereto or a current therethrough, the under layer is exposed and this under layer can then be used for transfer purposes.

Another object is to provide an improved method of recording and duplicating electric signals by subjecting a novel matrix or master record blank to the action of electric signals so as to expose the blank in successive elemental areas which areas are used for contact transfer purposes.

A still further object relates to an improved recording system employing a novel type of recording blank which may be used for multiple transfer operations.

A further feature relates to a novel method of producing an original message record blank and a large number of duplicates thereof without employing a photographic printing process.

A still further feature relates to the novel organization, arrangement and relative location and constitution of parts whereby there is produced an improved facsimile recording and duplicating blank.

Other features and advantages not specifically enumerated will be apparent after a consideration of the following detailed descriptions and the appended claims.

25 While the invention will be described herein in connection with a telefacsimile recording blank, it will be understood that this is done merely for explanatory purposes. Accordingly in the drawing,

30 Fig. 1 represents an enlarged cross section of part of one form of recording blank embodying principles of the invention.

Fig. 2 represents a modification of the blank of Fig. 1.

35 Fig. 3 is a diagrammatic view of a facsimile recording and duplicating system embodying features of the invention.

Fig. 4 is an enlarged perspective view of a modified record blank.

40 Referring to Fig. 1, the facsimile recording blank according to the invention is shown as comprising a base or carrier 1 of paper, although other pliable materials such as fabric, photographic transparencies or the like may be employed.

45 The paper 1 is provided with a stratified sheath comprising two strata or layers 2, 3. Layer 2 is especially designed so that in addition to having a desired electrical conductivity, it also acts as a retainer for a dye or dyes which control

50 the subsequent duplicating step. This recording and duplicating blank can be used to receive and record electric signals such as facsimile or telegraph signals by well-known telefacsimile procedure, either by means of an electric space discharge to or through the sheath, e. g., by means of a corona discharge, or by means of a current which is caused to flow conductively through the paper transverse to its cross section. The surface

of the record blank is, in accordance with well-known facsimile scanning methods, acted upon in successive areas of elemental size and in synchronism with a corresponding scanning process at the facsimile transmitter. Where the recording is effected by an electric space discharge, e. g., corona as described in Patent 1,702,595 to A. G. Cooley, it is not necessary that the base 1 be of conducting paper. In the current conducting type of record, it may be necessary that the base 1 be of conducting paper. It will be understood therefore, that the base paper 1 may be either non-conducting or substantially so, or it may be specially treated to render it of the desired conductivity in accordance with the particular type of electric current that is used for recording.

If paper 1 is of the non-conducting type, it may be a well-known white or colored paper upon which is applied a black conducting layer 2 comprising "gas black" together with a dye or dye mixture and a suitable binder or adhesive. We have discovered that "gas black" is particularly well suited to the formation of this conductive dye-carrier layer or coating. For convenience of description, the dye-carrier layer 2 will be referred to herein as the duplicating layer or coating. The outermost layer 3 which will be referred to herein as the facsimile coating, consists of a pigment, usually white, to contrast with the black layer 2, the pigment being incorporated with a suitable adhesive or binder.

The amount and kind of dye which, in accordance with the invention, is incorporated in layer 2, will depend upon the character and number of copies that are to be made from the master facsimile record blank. Almost any dye is suitable for incorporating in the black layer 2, the type of solvent used for the copying process and the desired color of the copies determining the type of dye to be selected. Dyes like crystal violet, methyl violet, basic fuchsin, methyl green, water soluble nigrosine, chrysoidin brown, etc., can be used in coatings of the type proposed in Examples I and III. Since nigrosine does not produce good copies or as large a number as would be obtained from an equal amount of crystal violet used in the formula for instance, mixture of dyes giving a good black color, i. e., a mixture of crystal violet, methyl violet, basic fuchsin and chrysoidine can be used as in Example III.

Oil or alcohol soluble dyes can be used in coatings of the type proposed in Example II.

The amount of dye to be used in coating 2 will vary with the type of dye and results desired. Anywhere from 10 to 150% based on the weight of gas black used will be satisfactory.

In using our invention as a facsimile paper a preferable conducting layer 2 comprises gas black mixed with any suitable adhesive such as gelatin, gum, starch, casein, emulsified wax, cellulose ether or ester, etc., and a suitable dye. The amount and kind of the binder used has a pronounced effect on the recording properties of the paper. In the case of binders of any of the types mentioned above it is desirable to use as little binder as possible and in general the amount of binder may vary from five to thirty percent of the dry weight of the gas black. It may be said in general that it is preferable to use such binders as gelatin, gum, starch, casein, emulsified wax or the like materials for the black conducting coating 2 and to use binders of the cellulose ester or ether type for the white or facsimile coating 3, because if the same type of binder is used for both

coatings there will be a tendency for the two coatings to mingle when the facsimile coating 3 is applied, which is extremely undesirable. Also it is necessary to select the proper combination of binders and solvents for both coatings so that the dye of coating 2 will be very soluble in its solvent and will be well distributed when dry but will not mingle with the facsimile coating 3 when it is applied. If the binder of the black coating is of the cellulose ester or ether type, methyl cellulose is an exception, then the facsimile coating binder should be of the gelatin, gum, starch, casein, etc., type. However, these gelatin, gum, starch, casein binders are generally soluble in water and the paper would, if they were used as binders for the facsimile coating, be subject to water spotting and smearing due to handling.

As examples of the proportions of gas black, dye and binder which may be utilized in forming conducting coatings for facsimile papers of the type of our invention, the following are given:

#### Example I

|                                                                      |       |      |
|----------------------------------------------------------------------|-------|------|
| Gas black (Dixie #5 manufactured by the United Carbon Company, Inc.) | grams | 5.0  |
| Methocel (15 c. p. s.; manufactured by the Dow Chemical Company)     | do    | 2.0  |
| Crystal violet                                                       | do    | 4.0  |
| Water                                                                | cc    | 55.0 |

The methocel is dissolved in a portion of the water and the gas black added while stirring. The dye is added to the remaining water and heated slightly to dissolve it completely. A small amount of glycerol, carbitol or the like material may be added to increase the solubility of the dye. The mixture is then passed through a colloid mill or similar device and applied to the paper by any of the normal coating methods, such as spraying, dipping, brushing, or knife coating, etc. After coating the paper the liquid contained in the binder is evaporated off by heating or any other suitable method. The paper may thereafter be subjected to calendering in order that the surface may be smooth.

#### Example II

|                                                                            |       |      |
|----------------------------------------------------------------------------|-------|------|
| Gas black (kosmos 15D; manufactured by the United Carbon Company, Inc.)    | grams | 7.0  |
| Cellulose nitrate lacquer (No. 1,151,287, manufactured by Valentine & Co.) | grams | 7.0  |
| Oil soluble nigrosine                                                      | do    | 6.0  |
| Lacquer solvent (No. 1,001,012, manufactured by Valentine & Co.)           | cc    | 50.0 |

In this instance the dye is dissolved in the lacquer solvent and the gas black and lacquer mixed therewith. The resulting product is passed through a colloid mill or similar device before application to the paper. The mixture may be applied to the paper by any of the methods mentioned in connection with Example I, and the steps of heating or otherwise evaporating off the liquid and of calendering will likewise be utilized as in Example I.

#### Example III

|                                                                                  |       |      |
|----------------------------------------------------------------------------------|-------|------|
| Gas black (Dixie #5 manufactured by the United Carbon Company, Inc.)             | grams | 5.0  |
| Polyvinyl alcohol (R. H. 488 manufactured by the E. I. Du Pont de Nemours & Co.) | grams | 1.2  |
| Crystal violet                                                                   | do    | 1.1  |
| Methyl green                                                                     | do    | 1.0  |
| Basic fuchsin                                                                    | do    | 0.4  |
| Chrysoidine                                                                      | do    | 1.5  |
| Water                                                                            | cc    | 55.0 |

In this instance a combination of dyes was selected to produce a black color. The polyvinyl alcohol is dissolved in a portion of the water and the gas black added. The dyes are dissolved in the remaining water by heating slightly and added to the black dispersion. Thereafter the mixture is passed through a colloid mill or similar device before application to the paper. The application may be by any of the methods suggested hereinabove, and of course, includes the steps of evaporating the liquid from the binder and of calendering if necessary.

For facsimile paper purposes the paper after coating with the first or conducting coating 2 is further processed with the second or facsimile coating 3. This latter coating consists of a white or light colored pigment and a binder. The binder utilized may be any one of those mentioned in connection with the conducting coating, but as has been stated it is preferable to utilize a binder soluble in organic solvents for the facsimile coating, and one soluble in water for the conducting coating. Amongst the pigments which are satisfactory for use in the facsimile coating may be mentioned zinc sulphide, zinc oxide, barium sulphate, barytes, blanc fixe, lithopone, titanium dioxide, and the like. The sensitivity of some of these pigments may be improved by incorporating in them a small percentage, approximately 0.2 to 1.0%, of either mercuric sulphide, red or yellow lead oxide, stannic sulphide, etc. Of course it must also be kept in mind to so select the solvent for the facsimile coating so that the ingredients from either coating will not mingle.

The amount of the facsimile coating necessary to produce a satisfactory recording paper is very small. The exact amount cannot be stated since variation in weight of the paper and variation in thickness of the black conducting coating will cause variations which make it difficult to measure. It may be said, however, that as little coating as possible should be applied; just sufficient to cover the black conducting coating uniformly and to give the finished surface a light gray appearance. It is desirable to apply the facsimile coating in such a manner as to retain the pigment on the surface of the black coating. In order that this may be accomplished it is desirable that the coating be dried quite rapidly.

Examples of satisfactory facsimile coatings together with solvents are set forth below.

#### Example IV

|                                                                 |       |       |
|-----------------------------------------------------------------|-------|-------|
| Zinc sulphide                                                   | grams | 40.0  |
| Methocel (15 c. p. s. manufactured by the Dow Chemical Company) | grams | 2.5   |
| Water                                                           | cc    | 100.0 |

The methocel is dissolved in cold water and the zinc sulphide added with stirring. The mixture is passed through a colloid mill or similar device and applied to the paper by any of the methods mentioned hereinabove. This type of coating is for use with black conducting coatings similar to those shown in Example II.

The mixture of the following Example V comprises a binder of cellulose derivative in an organic solvent having little affinity for water soluble dyes and is preferred as a coating for application over the black or conducting coating containing a water soluble binder such as those described in Examples I and III.

#### Example V

|                                                                                                                                                                                                                                          | Grams |
|------------------------------------------------------------------------------------------------------------------------------------------------------------------------------------------------------------------------------------------|-------|
| Zinc oxide                                                                                                                                                                                                                               | 60.0  |
| Mercuric oxide                                                                                                                                                                                                                           | 0.3   |
| 5 Lacquer base consisting of 10% B. R. 254 resin manufactured by the Bakelite Corporation, 75% Ethocel. 10 c. p. s. Standard; manufactured by the Dow Chemical Company and 15% of No. 6 plasticizer manufactured by the Dow Chemical Co. | 15.0  |
| Solvent consisting of 70% toluol and 30% ethyl acetate                                                                                                                                                                                   | 125.0 |

The lacquer base is dissolved in the solvent and the zinc oxide and mercuric oxide thereafter added. The mixture is then passed through a colloid mill or other similar device before application to the paper, which application may be by any of the methods herein mentioned.

#### Example VI

This example is similar to the above except that cellulose nitrate is used as the cellulose derivative.

|                                                                                                                                                                                                                  | Grams |
|------------------------------------------------------------------------------------------------------------------------------------------------------------------------------------------------------------------|-------|
| Zinc oxide                                                                                                                                                                                                       | 60.0  |
| Mercuric oxide                                                                                                                                                                                                   | 0.3   |
| 25 Lacquer base consisting of 15% ester gum 125 manufactured by the American Cyanamid & Chemical Corporation, 70% nitro cellulose 2 second and 15% of No. 6 plasticizer manufactured by the Dow Chemical Company | 18.0  |
| Solvent consisting of 70% toluol 25% ethyl acetate and 5% denatured alcohol                                                                                                                                      | 140.0 |

The lacquer base is dissolved in the solvent and the zinc oxide and mercuric oxide thereafter added. The mixture is prepared and applied by any of the methods herein mentioned.

40 Referring to Fig. 3, there is shown in generalized schematic form, a telefacsimile recording and duplicating system wherein the numeral 5 represents any well-known form of telefacsimile transmitter whereby the subject matter to be transmitted is scanned in successive areas of elemental size to produce corresponding electric signals. These signals are transmitted over a suitable transmission channel 6 to the facsimile receiver 7, the output of which energizes the recording needle 8 with a corona producing voltage whose effective recording value is determined by the received telefacsimile signals. The needle 8 is slightly spaced from the recording blank 9 which is carried by the rotating drum 10. The drum 10 is rotated and advanced longitudinally in any manner well-known in the facsimile scanning arts and in synchronism with the corresponding scanning equipment at the transmitter 5. The recording blank 9 is formed of a base 60 of paper having two superposed layers corresponding respectively to layers 2 and 3 of Fig. 1. As a result of the corona discharge from needle electrode 8, the outer or facsimile layer 3 is removed at the points corresponding to the original subject matter scanned at the transmitter 5 thus exposing the dye-carrying transfer layer 2. The subject matter is therefore directly produced on the blank 9 and this blank may be removed and its surface moistened by a suitable solvent for the dye in coating 2 but which solvent does not affect the coating 3. This moistened record blank can then be used as a matrix to transfer the recorded subject matter any desired number of times to any suitable receiving surface such as to a succession of paper sheets 11. The transfer of the

moistened dye-record from blank 8 to the copy sheets 11 can be done either directly as described, or indirectly by "Ditto" or "Hectograph" process. Thus the dye record on blank 8 can be transferred by contact with a hectograph blank 12 comprising an aqueous solvent held by a moistened gelatin-glycerol compound which receives the impression in reverse from the master record and transfers it to the paper or sheet material in readable form by bringing the two in contact with each other. Water is used as the solvent for the copying machine process and alcohol solutions for the spirit process.

The copying facsimile paper of this invention can be used to produce copies either from aqueous or alcoholic solvent processes and by proper selection of the dye in coating 2 and binder base in coating 3 can be made to operate using other solvents if occasion arises. Thus for example the black conducting coating of Example II covered with facsimile coating IV could be used to make copies using oil, toluol, acetone or the like as solvent and replacing the gelatin-glycerol compound with one adoptable to use with such solvents. The wide latitude offered by the copying facsimile paper of this invention is therefore quite obvious.

The number of copies that can be obtained from a single facsimile recording used as a master record is also very large, larger than for any known master records using the described method of copying, and a distinct feature of this particular combination of paper and coatings. This results from the fact that the master record holds or can be made to hold large quantities of dye and the master record can be used over and over again to produce fresh impressions on the gelatin-glycerol compound. Over 1,000 clear legible copies have been made from a facsimile recording.

It is possible by suitably plasticizing coating 3 in Example V or VI to produce a paper that could be used to make typewriter or telegraph printer records. In this case the characters of the typewriter or telegraph printer will perforate the coating 3 and expose the color bearing coating 2 leaving an impression of the character. The copying from such a record can then be made in the usual way. Of course a paper of this nature as illustrated by Fig. 2 need not contain the gas black of coating 2 but only the dye and binder.

Referring to Fig. 4, there is shown a modified form of record blank wherein the paper or base 15 is provided with a layer of chemical 16 such as iodine and this layer is covered with a facsimile coating 17 corresponding to coating 3 of Fig. 1. As the coating 17 is acted upon by the electric discharge or electric current corresponding to the facsimile electric signals, the chemical coating 16 is exposed. The copy paper 18 which is used with this facsimile blank has its surface of such chemical composition that when it contacts with the exposed iodine or chemical 16 at the recorded points of the blank, it changes the color of the surface of the copy paper 18. Thus the paper 18 may have incorporated in its body or surface a predetermined quantity of starch which reacts with the moistened exposed iodine

record 19 so as to change the color of the surface of the paper 18 in accordance with the facsimile record. While two typical methods of transferring the facsimile record have been disclosed, namely by a dye transfer, and by chemical interaction, it will be understood that other equivalent methods of transferring the record from the facsimile blank to the multiple copy sheets can be employed. Various changes and modifications may be made herein without departing from the spirit and scope of the invention.

This application is a division of application Serial No. 435,944, filed March 24, 1942, wherein the claims to the recording blank per se and process of preparation are presented.

What is claimed is:

1. The method of recording employing a recording blank of the type having an undercoating containing a transferable marking medium 20 and an overcoating therefor, which comprises generating electric signals representing the shades of successive elemental areas of the subject matter to be recorded, applying said signals to selected elemental areas of the overcoating to correspondingly expose the undercoating, and contacting the recording blank with a receiving surface to transfer to the latter a record only of the marking medium in said exposed areas.

2. The method according to claim 1 in which 30 the said transfer to the receiving surface is effected by a hectograph process.

3. The method according to claim 1 in which the said transfer is effected by a chemical interaction between said marking medium and the 35 recording surface.

4. The method of tele-recording employing a recording blank of the type having an undercoating containing a transferable dye and an overcoating, which comprises applying electric signal 40 potentials to selected elemental areas of the overcoating to correspondingly expose the undercoating, and contacting the recording blank with a receiving surface to transfer to the latter a record only of said exposed areas.

5. A recording system of the character described, comprising a source of electric signal impulses, a recording blank in the form of a pliable sheet having a double stratum coating with the understratum including a transferable dye, the overcoating being of a material which is removable in selected elemental areas in response to signals from said source applied thereto, and a receiving surface for contacting with said blank to transfer to the receiving surface a record only of those areas which have been acted upon by said potentials.

6. A recording system according to claim 5 in which said understratum also includes a material for imparting a desired electrical conductivity thereto.

7. A recording system according to claim 5 in which the pliable material has a base of non-conducting paper and means are provided for converting electric signals into a corona discharge acting on said elemental areas.

HAROLD R. DALTON,  
AUSTIN G. COOLEY.